

July 4, 1939.

H. C. PARKER ET AL

2,165,150

ARTICLE FOR CLEANING SHOES

Filed Oct. 8, 1935



Inventors

Henry C. Parker  
Elizabeth W. Parker

## UNITED STATES PATENT OFFICE

2,165,150

## ARTICLE FOR CLEANING SHOES

Henry C. Parker and Elizabeth W. Parker,  
Washington, D. C.

Application October 8, 1935, Serial No. 44,091

3 Claims. (Cl. 15—105)

This invention relates to article for cleaning shoes; and it comprises an article of rubber or the like adapted to be rubbed, for example, on a white shoe and impregnated with sufficient white pigment filler to leave a visible pigment mark when so rubbed; and it also comprises a method of cleaning white shoes, for example, wherein said article is rubbed on such a shoe until said shoe is cleaned and pigmented; all 10 as more fully set forth and as claimed.

The cleaning of pigmented shoes of the nature of white shoes has long presented a problem to the art. The lack of a suitable cleaning method has greatly restricted their use. The best cleaners which have thus far been developed comprise various aqueous suspensions of chalk and the like which are applied by means of a rag, sponge or brush. This procedure is supposed to clean as well as to whiten the shoes but the 20 amount of cleaning obtained is negligible. At best the dirty shoe is coated with a white chalky layer which poorly conceals its true condition and which, in time, flakes off. These cleaners cannot be applied uniformly and a streaked coating 25 is produced. The operation is extremely messy and time consuming. It is impossible to prevent the cleaner from reaching and soiling the sole of the shoe which is not supposed to be white and it is difficult to remove the cleaner from the sole. It is small wonder that shoe 30 shining parlors charge more for cleaning white and other pigmented shoes than for shoes of other colors.

Rubber is one of the most universally employed 35 cleaning agents. Rubber erasers have been used for fifty years or more. And it is not new to introduce sufficient filler into rubber erasers to produce slight tints. For example it has been suggested to introduce a greenish colored filler 40 into rubber erasers in order to imitate the color of writing paper and to counteract the usual smudge left upon erasure. Apparently it has never been suggested, however, to employ rubber in the cleaning of white shoes; that is, if the 45 use of sponge rubber applicators is excepted.

Ordinary rubber erasers are not satisfactory for the cleaning of white shoes owing to the fact that they are incapable of removing the stains which are produced when the shoes are worn in 50 the rain, for example. We have found, however, that when rubber is impregnated with sufficient white, chalk-like filler to make a distinct white mark when rubbed on a shoe a highly satisfactory cleaning and whitening action is produced. No 55 liquid is necessary, hence the operation is clean-

ly, and can be accomplished without soiling the hands. Moreover a rubber cleaner can be readily shaped to fit into the recess between the sole and the vamp, which is always difficult to reach with liquid cleaners. The cleaner can be constructed in such fashion that there is no danger of whitening the sole of the shoe. The rubber cleaner is inexpensive and the cleaning operation is easily and quickly accomplished.

We usually construct our rubber cleaner with 10 two ends connected with a hand grip. It is also advantageous to provide an attached brush for removing detached particles of rubber or for dusting off the shoes prior to cleaning. If desired 15 a scraper can also be provided. We usually shape the rubber ends in such manner that they are particularly adapted to fit the contour of the shoe. It is convenient to have the two ends of the cleaner of different rubber composition. 20 One end, for example may be of substantially pure rubber with the usual amount of fillers and can be used for cleaning where whitening is not required. It can also be used for removing any 25 white markings which may have been applied accidentally to the sole of the shoe. In any case 30 it is advantageous to have at least one edge made of ordinary rubber which can be used for cleaning without whitening. It is also desirable to provide a projecting corner or edge shaped to fit 35 into the recess between the sole and the vamp and in this case the edge which comes into contact with the sole can be made of ordinary rubber in order to prevent contamination of the sole.

In compounding the rubber used in my cleaner 35 for white shoes any of the usual whitening materials can be employed which are now used in the liquid cleaners. Prepared chalk, whiting, zinc white, white lead, barytes, titanium oxide 40 and the like are examples. Ordinarily the same pigment can be employed in the cleaner that is used in coloring the leather of the shoe during manufacture. The pigment is mixed with the rubber by milling in the ordinary way and is 45 employed in quantities sufficient to leave a distinct pigmented mark on the shoe. The exact proportions to be employed vary to some extent with the pigment which is used. The determination of suitable proportions is well within the 50 skill of the art. It will be found ordinarily that roughly twice the usual amount of filler used in making rubber erasers must be employed, say from 40 to 85 percent by weight, depending upon 55 the pigment used. The quantity should not

be so great, however, that the elasticity and strength of the rubber is greatly impaired.

In one specific example we added to a rubber mix, containing the usual vulcanizers, accelerators, etc., 75 per cent by weight of a zinc oxide-prepared chalk mixture, based on the weight of the composition as a whole. The mix was then thoroughly milled. This resulting mixture was molded and vulcanized in the usual way to form strips about 3 inches long and one-half inch thick. These strips were shaped at the ends and were found to be highly satisfactory as shoe cleaners. By rubbing these strips over a soiled white shoe, it was found that the shoe could be both cleaned and whitened.

In the accompanying drawing we have shown several illustrative embodiments of shoe cleaners of various shapes and styles within our invention.

In this showing:

20 Fig. 1 represents an elevational view of a double ended rubber cleaner.

Fig. 2 is a side view of the cleaner shown in Fig. 1,

Fig. 3 is an elevation of a single ended cleaner,

25 Fig. 4 is a side view of the cleaner of Fig. 3.

Fig. 5 shows a modification with a metal insert, while,

Fig. 6 shows a further modification.

In the various figures like parts are indicated by 30 like reference numerals. In Fig. 1 a metal casing 1 is shown, in one end of which is secured a rubber cleaner 2 having a white filler. At the other end a similar piece 3 of ordinary rubber is shown. A brush 4 is also mounted on one side of the casing 35 1. The rubber pieces 2 and 3 are roughly shaped to fit the curvature of a shoe as shown at 5. The projecting ends 7 and 8 are adapted to enter and clean the recess between the sole and the vamp. The edges may be merely blunt as shown at 9 or 40 may be tapered in arcuate manner as shown at 10, see Fig. 2.

The purpose of providing a portion 3 of the cleaner of ordinary rubber is to enable a person to clean the shoes before whitening. This has been 45 found to be an advantageous method of cleaning and whitening shoes. After the whitening operation, the detached particles of rubber may be brushed off if desired. To leave these particles on the shoe produces a duller finish.

50 In Fig. 2 an embodiment is shown wherein the rubber piece 3 has a concave face 10 roughly shaped to fit the contour of a shoe.

The embodiment shown in Figs. 3 and 4 is provided with a handle 11 with a brush 4 at one end and the cleaner 2 at the other. The handle 11 may be molded from any of the ordinary plastic compositions or may be hard rubber or metal. The cleaner 2 is provided with a strip 12 of rubber having a smaller amount of filler. This strip can 60 be obtained by applying a coating of rubber solution to this edge of the cleaner or this strip of rubber can be vulcanized to the larger piece of rubber containing white filler. The purpose of strip 12 is to prevent the sole of the shoe from 65 being marked during cleaning.

The cleaner of Figs. 3 and 4 is provided with a projecting corner 7 adapted to clean the recess between the sole and the vamp. It also has an

arcuate surface 13 which roughly fits the contour of the shoe.

In Fig. 5 a metal insert 15 is shown attached to one edge of the cleaner. This metal protects the sole from being marked. It also can be used as a 5 scraper. The metal can be secured to the rubber by known adhesives forming a tight joint.

In Fig. 6 a modification is shown in which two pieces of rubber are vulcanized together, one piece 2 containing pigment and the other piece 3 containing insufficient pigment to color the shoe. The cleaner is tapered to a point which comes at the 10 joint between the two rubber sections. Thus a pigmenting portion and a cleaning portion are provided. If point 9 is rubbed into the recess 15 between the sole and the vamp of a shoe the sole will not be whitened.

It is of course obvious that many other modifications can be made which fall within the scope of our invention. Various shapes and sizes of 20 cleaner may be used. It is not even necessary to employ a handle since the brush can be secured directly to the rubber. And a brush can be dispensed with in the cheaper forms. Various types of white fillers can be employed. Or if the shoes 25 are of colored suede a filler can be used which matches the color of the shoe. Thus a bronze colored filler can be used for cleaning bronze suede, etc. In this case a wire brush can be provided for brushing up the nap of the suede. Our 30 invention is thus applicable to the cleaning of all types of pigmented shoes, that is, shoes which require an application of pigment when cleaned. It is possible to employ the so-called synthetic 35 rubber and rubber substitutes in our invention in place of true rubber. The term "rubber" in the following claims is intended to cover such equivalents. Many other modifications within the scope of the following claims will be immediately evident to those skilled in the art.

What we claim is:

1. A cleaner for pigmented shoes comprising a piece of rubber having a projecting portion adapted to clean the recess between the sole and the vamp of a shoe and an adjacent arcuate section being a continuation of said projecting portion adapted to fit the contour of the vamp, said piece of rubber containing sufficient colored pigment to produce a visible pigmented mark when rubbed on a shoe.

2. The cleaner of claim 1 wherein one edge of said projecting portion is provided with means for protecting the sole of the shoe from pigment while being cleaned.

3. An article for cleaning and coloring pigmented shoes comprising a two-faced portion adapted to clean between the sole and the vamp of a shoe, one of said faces being adapted to be rubbed against the sole of said shoe without coloring the same and the directly opposed face being 60 adapted to be simultaneously rubbed against the vamp of said shoe; said latter face being composed of rubber having sufficient pigment compounded therewith to produce a visible colored mark on said shoe.

HENRY C. PARKER.  
ELIZABETH W. PARKER.